

# UNITED STATES PATENT OFFICE.

OTTO LIEBKNECHT, OF FRANKFORT-ON-THE-MAIN, GERMANY, ASSIGNOR TO THE ROESSLER & HASSLACHER CHEMICAL CO., OF NEW YORK, N. Y., A CORPORATION OF NEW YORK.

## ELECTROLYTIC PROCESS OF MAKING ALKALI PERBORATES.

1,268,369.

Specification of Letters Patent.

Patented June 4, 1918.

No Drawing.

Application filed October 23, 1915. Serial No. 57,396.

To all whom it may concern:

Be it known that I, OTTO LIEBKNECHT, a subject of the Emperor of Germany, residing at Frankfort-on-the-Main, Germany, have invented certain new and useful Improvements in Electrolytic Processes of Making Alkali Perborates, of which the following is a specification.

This invention relates to the art of making perborates and it relates particularly to a process for the electrolytic production of sodium perborate by an electrolytic process.

Perborates are usually manufactured by the well-known Tanatar method wherein oxygen is transferred to borates from any substance carrying oxygen in available form; such substances are for instance, hydrogen peroxid, sodium peroxid, and percarbonates of various origin.

The above substances, however, can only be obtained at a high price, nor are the perborates obtainable therefrom, producible at a sufficiently low price as is desirable in view of their meritorious properties.

It has been tried for a long time to obtain the same result by the electrolytic oxidation of a solution of a borate and to operate this process on a commercial scale by electrolyzing a mixed solution of an alkali borate and an alkali carbonate.

These efforts, however, met with considerable difficulties and a noteworthy success could not be achieved for the reason already recognized by Tanatar, who in *Zeitschrift fuer Physikalische Chemie*, vol. 29, page 162, makes the following statement: "The electrolytic current (electrolysis) also decomposes the perborates though the generation of small quantities of perborates is taking place during the electrolysis of concentrated solutions."

This important statement leaves no doubt that a considerable concentration of oxygen cannot be obtained by the electrolysis of a solution of borates, and that an equilibrium is reached very soon with a rather weak concentration of oxygen so that just as much perborate is decomposed as is generated.

I have now made the surprising observation that the electrolytic production of alkali perborates, as for instance of sodium

perborate, proceeds in a commercially successful manner if solid borax is present, preferably suspended, in the solution of alkali carbonate submitted to the action of the electric current, whereby unexpectedly, solid sodium perborate is directly obtained.

If I suspend for instance granulated borax, in a solution of soda, through which an electric current is passing, I succeed in a short time in proving active oxygen to be present in the precipitate *i. e.* sodium perborate has been generated. By duly continuing the electrolysis I succeed in transforming all the borax into a marketable sodium perborate of crystallized form. I thus obtain marketable, solid sodium perborate immediately in one single operation.

My invention offers also the further advantage of making any desired mixture of perborate and borax (perborax) by discontinuing the electrolysis at a given moment.

The reaction can also be accelerated by adding to the solution, certain agents, as for instance, sodium perborate, to which also sodium bicarbonate, or materials generating such, may be added.

In further investigating the reaction, I found it very much dependent upon the purity of the applied raw-materials. Impurities, often present in these materials, and known to be catalysts, as for instance iron-compounds, disturb the generation of solid perborate very considerably. If I electrolyze solutions carrying such impurities, a de-poisoning or self-purification by the effect of the electrolysis takes place only after a certain time, whereupon the normal generation of perborate continues. To avoid this disadvantage entailing a loss of energy, I apply such raw materials as are practically free from catalysts or I remove the catalysts from the raw materials; to achieve this latter purpose it is sufficient for instance in the case of applying a solution of Solvay-soda, containing almost always a certain quantity of iron compounds even after filtration, to boil such solution and to filter the same to obtain a solution suitable to serve as the electrolyte.

Finally I may also retard or entirely remove the harmful effect of the catalysts by adding to the electrolyte such materials

known to be negative catalysts exerting a protective action. The yields I obtain for instance with an unpurified solution of Solvay-soda, to which I add small quantities 5 of stannic acid, are equal to those obtained with a purified solution of soda; I am almost under the impression that these agents exert a protective action as well as a favorable effect thus recommending their application 10 also in the use of raw materials practically free from catalysts. Sodium perborate or similar materials work in the same direction, as their addition counteracts the effect of the catalysts. The favorable effect of these 15 agents is even enhanced by the presence of several of the same.

In the practical operation of my invention 20 I have found that the density of current may vary within a very great range; for instance I may work with a density of 2000 amp. per square meter as well as with one half or double this density; the temperature may likewise vary within a great range. However, I have found the temperature of 13° C. 25 very suitable for the process.

In using the expression "granulated borax" both in the specification and claims, I mean to include borax sufficiently finely divided for the purpose in hand although in 30 practice I prefer to use borax in such finely divided state that it is substantially dust-like.

I claim:

1. The process of making alkali perborates, consisting in electrolyzing a solution 35 of an alkali carbonate in the presence of a solid alkali borate.

2. The process of making alkali perborates, consisting in electrolyzing a solution 40 of an alkali carbonate in the presence of a solid granulated alkali borate, said alkali borate being suspended in the solution of the alkali carbonate.

3. The process of making alkali perborates, consisting in rendering a solution of 45 an alkali carbonate substantially free from catalyzing substances, maintaining a solid granulated alkali borate free from catalyzing substances suspended in said solution and electrolyzing the solution containing the solid alkali borate in suspension.

4. The process of making alkali perborates, consisting in preparing a solution of 55 an alkali carbonate previously rendered free from catalysts, maintaining a solid granulated alkali borate previously rendered free from catalysts suspended in said solution and electrolyzing the solution containing the solid alkali borate in suspension.

- 60 5. The process of making alkali perborates, consisting in preparing a solution of an alkali carbonate, maintaining a solid granulated alkali borate suspended in said solution, adding to the mixture substances 65 adapted to counteract the effect of catalysts

contained in the aforesaid solution of alkali salts and electrolyzing the solution containing the solid alkali borate in suspension.

6. The process of making alkali perborates, consisting in preparing a solution of 70 an alkali carbonate, maintaining a solid granulated alkali borate suspended in said solution and electrolyzing the solution in the presence of substances accelerating the reaction.

7. The process of making alkali perborates, consisting in preparing a solution of an alkali carbonate, maintaining a solid 80 granulated alkali borate suspended in said solution and electrolyzing the solution in the presence of a plurality of metallic compounds accelerating the reaction.

8. The process of making alkali perborates, consisting in preparing a solution of an alkali carbonate, maintaining a solid 85 granulated alkali borate suspended in said solution and electrolyzing the solution in the presence of a mixture of an alkali bicarbonate, an alkali perborate and stannic acid to accelerate the reaction.

9. The process of making alkali perborates, consisting in preparing a solution of alkali carbonate, maintaining a solid granulated alkali borate suspended in said solution and electrolyzing the solution in the 95 presence of an alkali bicarbonate to accelerate the reaction.

10. The process of making alkali perborates, consisting in preparing a solution of alkali carbonate, maintaining a solid granulated alkali borate suspended in said solution and electrolyzing the solution in the presence of an alkali perborate to accelerate the reaction.

11. The process of making alkali perborates, consisting in preparing a solution of alkali carbonate, maintaining a solid granulated alkali borate suspended in said solution and electrolyzing the solution in the presence of a mixture of an alkali perborate 105 and an alkali bicarbonate to accelerate the reaction.

12. The process of making alkali perborates, consisting in preparing a solution of alkali carbonate, maintaining a solid granulated alkali borate suspended in said solution, counteracting the effect of catalyzing substances by adding stannic acid to the mixture and then electrolyzing the latter.

13. The process of making sodium perborate, consisting in electrolyzing a solution of soda in the presence of solid borax.

14. The process of making sodium perborate, consisting in electrolyzing a solution of soda in the presence of solid granulated borax, said granulated borax being suspended in the solution of the soda.

15. The process of making sodium perborate, consisting in rendering a solution of soda substantially free from catalyzing sub- 130

stances, maintaining solid granulated borax free from catalyzing substances suspended in said solution and electrolyzing the solution containing the solid borax in suspension.

16. The process of making sodium perborate, consisting in preparing a solution of soda previously rendered free from catalysts, maintaining solid granulated borax previously rendered free from catalysts suspended in said solution and electrolyzing the solution containing the solid borax in suspension.

17. The process of making sodium perborate, consisting in preparing a solution of soda, maintaining solid granulated borax suspended in said solution and electrolyzing the same in the presence of a mixture of sodium bicarbonate, sodium perborate and

20 stannic acid to accelerate the reaction.

18. The process of making sodium perborate, consisting in preparing a solution of soda, maintaining solid granulated borax suspended in said solution and counteracting 25 the effect of catalysts by adding stannic acid to the mixture while electrolyzing the latter.

19. The process of making sodium perborate, consisting in preparing a solution of soda, maintaining solid granulated borax 30 suspended in said solution and electrolyzing the solution in the presence of sodium bicarbonate to accelerate the reaction.

20. The process of making sodium perborate, consisting in preparing a solution of 35 soda, maintaining solid granulated borax suspended in said solution and electrolyzing the solution in the presence of sodium perborate to accelerate the reaction.

21. The process of making sodium perborate, consisting in preparing a solution of soda, maintaining solid granulated borax suspended in said solution and electrolyzing the solution in the presence of a mixture of sodium bicarbonate and sodium perborate to 45 accelerate the reaction.

In testimony whereof I have signed this specification in the presence of two subscribing witnesses.

OTTO LIEBKNECHT.

Witnesses:

JEAN GRUND,  
CARL GRUND.